

## UNITED STATES PATENT OFFICE

2,206,846

## ALLOY STEEL

Clarence H. Lorig, Columbus, Ohio, assignor to  
Battelle Memorial Institute, Columbus, Ohio, a  
corporation of Ohio

No Drawing. Application July 11, 1938,  
Serial No. 218,633

## 5 Claims. (Cl. 75—125)

My invention relates to an alloy steel. It relates more particularly to a steel which has a high sensitivity to work-hardening.

One of the objects of this invention is the provision of an alloy steel which may be used for producing wrought and cast articles having a high capacity for work-hardening.

A further object of this invention is the provision of an alloy steel used for producing articles having a high sensitivity to work-hardening that possesses great strength and toughness.

Still another object of this invention is the provision of a work-hardenable alloy steel product having great strength and toughness.

Other objects and advantages of my invention will become apparent from the following description and claims.

I have found that the manganese content of the 11 to 14 per cent manganese work-hardening steel can be substantially reduced by alloying with copper and molybdenum and that the stabilization of the austenite structure of this type of work-hardening steel can be accomplished by employing much lower manganese contents when both copper and molybdenum are present. The composition range in which the specified advantages were found is as follows:

Carbon 0.50 to 1.7 per cent, manganese 2.0 to 9.0 per cent, copper 1 to 5 per cent, molybdenum traces to 3.0 per cent, the remainder being iron together with the usual amounts of silicon, sulfur, and phosphorus normally in steel. From traces up to 0.15 per cent phosphorus, from traces

up to 0.10 per cent sulfur, and from traces up to 1.5 per cent silicon may be present in the steel. Some chromium may be used to further increase the wear resistance and to raise the yield and tensile strengths of the steel. For this purpose, however, less than 3 per cent of chromium is satisfactory.

I have discovered the combining of manganese, copper, molybdenum, and carbon in the proportions indicated makes steel very sluggish to allotropic changes, so that in the water-quenched condition or after cooling quickly in air it stays in the austenitic state. However, the changes are not too sluggish, so that cold-working will cause the worked surface of the steel to transform from soft austenite to extremely hard martensite. High sensitivity to work-hardening is obtained when the transformation of austenite to martensite by cold working is rapid. In applications where my steel is subjected to combined pounding or impact and abrasion, the transformation is rapid and the steel resists wear to a remarkable degree. New, hard surfaces form as rapidly as the earlier martensitic surfaces are removed by wear.

The following table lists the hardness of a number of steels after different heat treatments and shows the relative work-hardenability of the steels by the difference in Rockwell "C" hardness of the unworked surface and the hardness at the bottom of a Brinell impression where the metal is worked.

| Steel No. | C, per cent | Mn, percent | Cu, percent | Mo, percent | Hardness after various heat treatments |              |                                      |                     |              |                                      |                         |              |                                      |
|-----------|-------------|-------------|-------------|-------------|----------------------------------------|--------------|--------------------------------------|---------------------|--------------|--------------------------------------|-------------------------|--------------|--------------------------------------|
|           |             |             |             |             | 1650° F. water quenched                |              |                                      | 1650° F. air cooled |              |                                      | 1650° F. furnace cooled |              |                                      |
|           |             |             |             |             | Brinell hardness                       | Rockwell "C" |                                      | Brinell hardness    | Rockwell "C" |                                      | Brinell hardness        | Rockwell "C" |                                      |
|           |             |             |             |             |                                        | Sur-<br>face | Bottom of<br>Brinell im-<br>pression |                     | Surface      | Bottom of<br>Brinell im-<br>pression |                         | Sur-<br>face | Bottom of<br>Brinell im-<br>pression |
| 45 1      | 0.5         | 1.5         | 3.0         | 0.5         | 578                                    | 61           | 67                                   | 549                 | 55           | 60                                   | 361                     | —            | 45                                   |
| 2         | 1.2         | 3.0         | 3.0         | 0.5         | 200                                    | 24           | 43                                   | 210                 | 24           | 43                                   | 477                     | —            | —                                    |
| 3         | 1.2         | 3.0         | 3.0         | 3.0         | 232                                    | 32           | 46                                   | 241                 | 29           | 44                                   | 531                     | —            | —                                    |
| 4         | 1.2         | 2.0         | 5.0         | 1.0         | 245                                    | 35           | 56                                   | 285                 | 39           | 52                                   | 477                     | —            | —                                    |
| 5         | 1.25        | 2.0         | 3.0         | 0.5         | 255                                    | 33           | 50                                   | 401                 | 42           | 52                                   | 409                     | 39           | 44                                   |
| 6         | 1.25        | 4.0         | 4.0         | 0.5         | 224                                    | 19           | 34                                   | 242                 | 20           | 39                                   | 518                     | 49           | 54                                   |
| 7         | 1.25        | 5.0         | 3.0         | 0.5         | 217                                    | 14           | 28                                   | 228                 | 15           | 36                                   | 454                     | 33           | 49                                   |
| 8         | 1.25        | 5.0         | 3.0         | 0.75        | 229                                    | 23           | 36                                   | 232                 | 18           | 41                                   | 429                     | 43           | 50                                   |
| 9         | 1.25        | 6.0         | 3.0         | Trace       | 221                                    | 22           | 38                                   | 225                 | 20           | 42                                   | 404                     | 41           | 47                                   |
| 10        | 1.25        | 7.0         | 3.0         | Trace       | 228                                    | 24           | 40                                   | 246                 | 24           | 46                                   | 385                     | 38           | 46                                   |
| 11        | 1.25        | 7.0         | 3.0         | 0.50        | 229                                    | 23           | 39                                   | 229                 | 18           | 40                                   | 378                     | 40           | 54                                   |
| 12        | 1.25        | 7.0         | 1.5         | 0.50        | 224                                    | 18           | 38                                   | 241                 | 18           | 42                                   | 308                     | 39           | 55                                   |
| 13        | 1.25        | 4.0         | 1.0         | 0.50        | 226                                    | 20           | 35                                   | 256                 | 21           | 43                                   | 518                     | 49           | 54                                   |
| 14        | 1.25        | 4.0         | 2.0         | 1.00        | 229                                    | 20           | 34                                   | 232                 | 16           | 40                                   | 560                     | 52           | 58                                   |
| 15        | 1.50        | 3.0         | 3.0         | 0.5         | 269                                    | 28           | 43                                   | 354                 | 33           | 46                                   | 499                     | 49           | 54                                   |
| 16        | 1.00        | 3.0         | 3.0         | 0.5         | 215                                    | 27           | 42                                   | 205                 | 20           | 44                                   | 518                     | 50           | 54                                   |
| 17        | 0.75        | 3.0         | 3.0         | 0.5         | 477                                    | 54           | 60                                   | 435                 | 50           | 56                                   | 514                     | 52           | 54                                   |
| 18        | 1.25        | 5.0         | 3.0         | 0.25        | 224                                    | 18           | 39                                   | 234                 | 16           | 41                                   | 441                     | 42           | 51                                   |

As compared with the above steels, a 14 per cent manganese, 1.25 per cent carbon steel after quenching in water from 1900° F. had a Brinell hardness of 175, a Rockwell "C" hardness of 13 on the unworked surface, and a Rockwell "C" hardness of 40 on the bottom of a Brinell impression.

Water-quenched specimens of steel coming within the range of composition which I previously specified will have a Brinell hardness in excess of 210. In the range of composition centering around 1.00 to 1.5 per cent carbon, 3 to 7 per cent manganese, 1 to 4 per cent copper, and from traces to 1.00 per cent molybdenum, which is my preferred range, Brinell hardnesses of water-quenched specimens are from 210 to about 260, or values that are substantially above the value for the 14 per cent manganese steel. The higher hardness is also associated with higher tensile strength. In this range of preferred composition, the steel transforms very rapidly at the surface from soft austenite to extremely hard martensite on cold working, as shown by the difference in Rockwell "C" hardness of the un-worked surface and of the bottom of the Brinell impression of water-quenched material. The air-cooled steel in the same range of composition is also austenitic and also transforms to martensite on cold-working. After furnace cooling, the steel is partially or fully martensitic and hard.

Below the preferred range of carbon and alloy contents, it is more difficult to obtain the steel in the austenitic state and thus make it work-hardenable without an extremely drastic quenching from high temperatures.

Carbon has a very powerful influence on stabilizing austenite and in making the steel suitable for work-hardening. With carbon contents below 1.0 per cent, it becomes increasingly difficult to develop work-hardening properties in the steel. A suitable carbon range is quite narrow, as I have found that with carbon contents above 1.50 per cent the steel not only becomes harder in the quenched state but becomes less satisfactory for work-hardening. Carbon is, therefore, an important element which must be kept within close limits in my steel.

Copper and molybdenum augment carbon and manganese in retaining austenite. Both copper and molybdenum retard the rate of transformation of gamma iron to alpha iron, and particularly so in the presence of manganese and carbon. Consequently, I have found it possible to reduce the manganese in austenitic work-hardening steel as much as 75 per cent by alloying with copper and molybdenum. 1 to 5 per cent copper and from traces to 3 per cent molybdenum make possible a reduction in the amount of manganese of from 1 to 3 times the total percentage of copper and molybdenum added. Too high a molybdenum content like too high a carbon content tends to harden the steel when water-quenched, making it less susceptible to work-hardening. For that reason, I prefer to limit its use below 3 per cent. Excellent results are obtained with 0.25 per cent to 0.50 per cent molybdenum.

In addition to its influence on stabilizing austenite, copper increases the strength of the steel. In the range of composition in which the steel is machinable, copper also aids the machinability.

An important advantage of my alloy steel over the high-manganese steel is that in the range of composition of about 2 to 4 per cent of copper, 5 to 7 per cent of manganese, traces to 0.50 per

cent of molybdenum, and 1.00 to 1.50 per cent of carbon the steel is machinable with ordinary carbon and high-speed steel tools. The machinability of the steel in this range of composition constitutes quite an advance in the art, as the high-manganese steel can be machined only with the greatest difficulty by special carbide tools or by grinding. To effect machinability, the steel is cooled slowly as, for example, in a well-insulated furnace. The following table shows the maximum permissible machining speed for a number of compositions after they were cooled slowly in a furnace from 1650° F. Cuts were made on a lathe using a high-speed tool at a feed of  $\frac{1}{16}$ -inch per revolution. A specimen  $\frac{7}{8}$ -inch square was reduced to  $\frac{3}{4}$ -inch round in one cut.

| C, percent | Mn, percent | Mo, percent | Cu, percent | Brinell hardness | Maximum permissible machining speed, R. P. M. |
|------------|-------------|-------------|-------------|------------------|-----------------------------------------------|
| 1.25       | 3.0         | Trace       | 3.0         | 321              | 167                                           |
| 1.25       | 6.0         | Trace       | 3.0         | 406              | 100                                           |
| 1.25       | 7.0         | Trace       | 3.0         | 380              | 120                                           |
| 1.25       | 5.0         | Trace       | 3.0         | 415              | 87                                            |
| 1.25       | 2.0         | 0.5         | 3.0         | 415              | 45                                            |

After machining, the steel can be made work-hardenable by heat-treating and liquid or air-quenching.

The higher quenching temperatures up to a certain maximum were found to improve the ductility of the steel considerably. A quenching temperature above 1800° F. was found to be most satisfactory, although it is possible to quench from lower temperatures.

Mechanical properties of the steel in the preferred range of composition are excellent. Its toughness was demonstrated with key-hole notched Charpy specimens water-quenched and tested for impact in a machine of 120 ft.-lb. capacity. The specimens absorbed the full 120 ft.-lb. of energy of the machine with a single blow without breaking. Any steel coming within the range of composition specified hereinbefore will have an impact strength in excess of 30 ft.-lbs.

The alloy steel is suitable for services requiring high resistance to the combination of repeated blows or impact and abrasion. Articles such as plates for jaw crushers, ball mill liners, roll shells, dipper teeth, caterpillar shoes, etc., can be made from my alloy.

Having thus described my invention, what I claim is:

1. An alloy steel consisting of 0.50 to 1.7 per cent carbon, 2.0 to 9.0 per cent manganese, 1 to 5 per cent copper, traces to 3 per cent molybdenum, traces to 0.15 per cent phosphorus, traces to 0.10 per cent sulfur, traces to 1.5 per cent silicon, and the balance substantially all iron, said steel being austenitic after quenching from a high temperature.

2. An alloy steel consisting of 1.00 to 1.5 per cent carbon, 3 to 7 per cent manganese, 1 to 4 per cent copper, traces to 1.00 per cent molybdenum, traces to 0.15 per cent phosphorus, traces to 0.10 per cent sulfur, traces to 1.5 per cent silicon, and the balance substantially all iron.

3. An alloy steel containing 0.50 to 1.7 per cent carbon, 2.0 to 9.0 per cent manganese, 1 to 5 per cent copper, traces to 3 per cent molybdenum, traces to 0.15 per cent phosphorus, traces to 0.10 per cent sulfur, traces to 1.5 per cent silicon, and

the balance substantially iron, said steel being austenitic and work-hardenable after quenching from a high temperature and having a Brinell hardness in excess of 210 and an impact strength in excess of 30 ft.-lbs.

5. An alloy steel containing 1.00 to 1.5 per cent carbon, 3 to 7 per cent manganese, 1 to 4 per cent copper, traces to 1.00 per cent molybdenum, traces to 0.15 per cent phosphorus, traces to 0.10 per cent sulfur, traces to 1.5 per cent silicon, and the balance substantially iron, said steel being

austenitic and work-hardenable after quenching from a high temperature and having a Brinell hardness ranging from 210 to 260 and having an impact strength in excess of 120 ft.-lbs.

5. An alloy steel consisting of 1.00 to 1.5 per cent carbon, 3 to 7 per cent manganese, 1 to 4 per cent copper, 0.25 to 0.50 per cent molybdenum, traces to 0.15 per cent phosphorus, traces to 0.10 per cent sulfur, traces to 1.5 per cent silicon, and the balance substantially all iron. 10

CLARENCE H. LORIG.